

## UNITED STATES PATENT OFFICE.

WILLIAM RINTOUL AND DONALD CROSS, OF STEVENSTON, SCOTLAND, ASSIGNEES TO  
NOBEL'S EXPLOSIVES COMPANY, LIMITED, OF STEVENSTON, SCOTLAND.

## EXPLOSIVE

1,310,489.

No Drawing.

Application filed December 4, 1917. Serial No. 205,408.

Specification of Letters Patent. Patented July 22, 1919.

To all whom it may concern:

Be it known that we, WILLIAM RINTOUL and DONALD Cross, both subjects of the King of Great Britain and Ireland, residing at 5 Ardeer Factory, Stevenston, Ayrshire, Scotland, have invented certain new and useful Improvements in Explosives, of which the following is a specification.

This invention relates to the manufacture 10 of blasting explosives containing nitroglycerin and gelatinized nitrocellulose, and in which the ratio of nitroglycerin to nitrocotton is large.

In our prior United States applications 15 Serial Numbers 192,963 and 192,964, filed September 24, 1917, we have described the manufacture of certain improved blasting explosives in the cold, by the use of a small proportion of the order of 0.1 to 1 per cent. 20 of certain gelatinizing accelerants.

It is in some cases desirable to obtain the maximum output from a given plant. This can be attained by this invention with decreased risks as compared with present methods of manufacture by reason of the shorter time of incorporation required. We find that an increased output can be obtained by the utilization of small proportions of the order of 0.1 to 1 per cent. of certain of the 25 classes of substances described in our prior applications, and using elevated temperatures *e. g.*, the usual service method of working, *viz.*, 60° C. to 70° C., the increased output arising from the fact that the time required for gelatinization is greatly reduced.

The invention therefore consists in employing in the manufacture of blasting explosives a small proportion of the order of 0.1 to 1 per cent. calculated on the nitroglycerin of one or more members of the following classes, the gelatinization being effected with elevation of temperature, preferably such as is employed in the usual service method of making blasting gelatin and like 40 explosives, *viz.*, about 60° C. to 70° C.:

1. Urethanes, or esters of carbaminic acid.
2. Anilids.
3. Substituted ureas.
4. Condensation products of glycerol and 50 other polyhydric alcohols with aldehydes.
5. Homologues of oxanilic ester.
6. Aromatic bodies soluble in nitroglycerin, *e. g.*, mono-, di- or tri-nitrotoluene, mono-nitro-naphthalene, di-nitro-benzene, 55 nitro-xylenes, or mixtures of these bodies.

The above-mentioned organic bodies and their chemical equivalents for the purposes of this invention, or mixtures thereof, are herein collectively referred to as organic accelerants for the gelatinization. 60

Some of these, including those numbered from 1 to 5 inclusive, are both accelerants of gelatinization and stabilizers.

In carrying this invention into effect in one form, we dissolve a small quantity of 65 one of the above accelerating agents in the nitroglycerin in a proportion varying from 0.1 to 1 per cent. calculated on the nitroglycerin, according to the gelatinizing power of the particular substance selected, which must 70 be determined experimentally in each case. We stir the nitrocellulose into the nitroglycerin solution, add the other ingredients, if any, and complete the mixing in the usual manner, employing the ordinary elevation 75 of temperature of the usual service method, *viz.*, 60° C. to 70° C., and we find that a good blasting explosive is thus prepared in a shorter time than has hitherto been possible.

We find that while ordinary blasting gelatin of the following composition, *viz.*, 80

|                   |       |
|-------------------|-------|
| Nitroglycerin     | 90.6% |
| Nitro-cotton      | 8.8%  |
| Calcium carbonate | 0.6%  |

prepared by the usual service method at 50° C. to 70° C. requires about 75 minutes for gelatinization, the corresponding modified blasting gelatin of the following composition, *viz.*, 90

|                        |       |
|------------------------|-------|
| Nitroglycerin          | 91.6% |
| Soluble nitrocellulose | 7.5%  |
| Formanilid             | 0.2   |
| Form-o-toluidid        | 0.1   |
| Calcium carbonate      | 0.6%  |

and prepared by the usual service method at 60° C. to 70° C., has the gelatinization completed in 30 minutes.

Again in the case of a gelignite, if an ordinary gelignite of the following composition, *viz.*:

|                   |       |
|-------------------|-------|
| Nitroglycerin     | 61.1% |
| Nitro-cotton      | 3.8%  |
| Wood meal         | 7.2%  |
| Potassium nitrate | 27.6% |
| Calcium carbonate | 0.3%  |

be prepared by the usual service method at 60° C. to 70° C., it requires about 75 minutes 110

for gelatinization; while a modified gelignite of the following composition, viz:

|                        |       |
|------------------------|-------|
| Nitroglycerin          | 60.8% |
| Soluble nitrocellulose | 3.8%  |
| Potassium nitrate      | 27.6% |
| Wood meal              | 7.2%  |
| Formanilid             | 0.2}  |
| Form-o-toluidid        | 0.1}  |
| Calcium carbonate      | 0.3%  |

and prepared by the usual service method at 60° C. to 70° C.; completes gelatinization in about 35 minutes:

The following are further examples of typical explosives which may be prepared according to this invention at the usual elevated temperatures, and containing aromatic nitro bodies soluble in nitroglycerin:

|     |                        |       |
|-----|------------------------|-------|
| I.  | Nitroglycerin          | 89.8% |
|     | Soluble nitrocellulose | 8.7%  |
|     | Liquid trinitrotoluene | 0.9%  |
|     | Calcium carbonate      | 0.6%  |
| II. | Nitroglycerin          | 60.5% |
|     | Soluble nitrocellulose | 3.8%  |
|     | Potassium nitrate      | 27.6% |
|     | Wood meal              | 7.2%  |
|     | Liquid trinitrotoluene | 0.6%  |
|     | Calcium carbonate      | 3%    |

The reduced times required for gelatinization of these compositions correspond very closely to those above indicated respectively.

The greatly reduced times of gelatinizing thus required are of great benefit from the point of view of reduction of the manufacturing risks as compared with present processes, as these risks practically vary proportionally with the time of working.

Again, reduced times of gelatinizing have the effect of lowering the average temperature attained by the mass during incorporation, and thus tend to increased safety.

Having now fully described and ascertained our said invention and the manner in which it is to be performed, we declare that what we claim is:

1. The manufacture of blasting explosives containing nitroglycerin and gelatinized nitrocellulose, consisting in incorporating a proportion of the order of 0.1 to 1 per cent. calculated on the nitroglycerin, of an organic accelerant for the gelatinization, the gelatinization being effected with elevation of temperature, the time factor of incorporation being thereby reduced, substantially as described.

2. The manufacture of blasting explosives containing nitroglycerin and gelatinized nitrocellulose, by dissolving in the nitro-glycerin prior to incorporation with the nitrocellulose a small proportion of the order of 0.1 to 1 per cent. calculated on the nitroglycerin of an organic accelerant for the gelatinization, and incorporating the other ingredients with this solution at an elevated temperature, whereby the time factor of gelatinization is reduced.

3. In the manufacture of blasting explosives, as claimed in claims 1 and 2, the utilization of an organic accelerant for the gelatinization which possesses also stabilizing properties.

In testimony whereof we have signed our names to this specification.

WILLIAM RINTOUL.  
DONALD CROSS.